

March 21, 1961

N. F. BAIRD

2,975,556

HEAT-PROTECTIVE COATING

Filed Sept. 24, 1957

FIG. 1.



FIG. 4.



FIG. 2.



FIG. 3.



FIG. 5.



FIG. 6.



FIG. 7.



INVENTOR.  
NORMAN F. BAIRD.  
ATTORNEY.  
J. V. Kelly

1

2,975,556

## HEAT-PROTECTIVE COATING

Norman F. Baird, Bloomfield, N.J., assignor to Westinghouse Electric Corporation, East Pittsburgh, Pa., a corporation of Pennsylvania

Filed Sept. 24, 1957, Ser. No. 685,865

6 Claims. (Cl. 49—78)

This invention relates to heat-protective coatings and, more particularly, to heat-protective coatings for processing aluminum base shells for lamps.

Incandescent lamp bases are prepared by first stamping a base shell into a predetermined configuration which is normally generally cylindrical and threaded, terminating in an inwardly-projected lip at the lower extremities of the base shell. This base shell forms one electrical contact for the lamp. An eyelet which is fabricated of an electrically-conductive material such as brass is positioned in a centrally-disposed location adjacent the lower extremities of the base shell proper, and this eyelet is electrically insulated from the base shell by an insulating button such as glass. This eyelet forms a second electrical contact for the incandescent lamp. In the normal procedures of fabricating the lamp base, the eyelet and base shell are placed into a mold and molten glass is inserted or poured into the lower interior surfaces of the base shell and about the eyelet. This electrically insulates the eyelet from the base shell and serves to secure the eyelet in a centrally-disposed position adjacent the lower extremities of the base shell.

In the practices of the prior art, the base shells were normally fabricated of brass. In recent years, the increased costs of brass have made it economically desirable to substitute aluminum in place of the brass. This substitution of aluminum has the disadvantage that the aluminum base shell has a tendency to melt somewhat during the so-called glassing operation when the molten glass is poured into the base shell. The melted aluminum sometimes forms a low-resistance path between the eyelet and the base shell, thereby shorting out the lamp, and the melted aluminum is also objectionable from the standpoint of appearance. While the primary purpose of an incandescent lamp is to convert electrical energy into light, the esthetic appearance of the lamp in the unburned condition is also a factor in promoting its initial sale to the user so that the maintenance of the base shell in as pleasing an appearance as possible is of great importance.

In order to overcome the foregoing and other difficulties of and objections to the prior art, it is the general object of this invention to provide a heat-protective coating for processing aluminum base shells in order to prevent any melting of the aluminum base shell.

It is a further object to provide a method for glassing an aluminum base shell for a lamp wherein any tendency of the aluminum to melt during the glassing operation is substantially inhibited.

It is another object to provide a method for glassing an aluminum base shell for a lamp wherein thinner base shells may be used.

The aforesaid objects of the invention, and other objects which will become apparent as the description proceeds, are achieved by providing a heat-protective coating for processing aluminum base shells, which coating principally comprises an admixture of sodium borophos-

2

phate and sodium polyacrylate in a water vehicle, wherein the constituents of the coating are maintained within permissible ranges and preferably at about a preferred concentration. In addition, there has been provided a method for glassing an aluminum base shell for a lamp where-

in the foregoing coating is first applied to the base shell before the glassing operation in order substantially to inhibit any tendency of the aluminum base shell to melt.

For a better understanding of the invention, reference

10 should be had to the accompanying drawing, wherein:

Fig. 1 is an elevational view of a completed incandescent lamp incorporating an aluminum base;

Fig. 2 is a sectional elevation of an unprocessed aluminum base shell;

Fig. 3 is a perspective view of an electrically-conducting eyelet before incorporation into the lamp base;

Fig. 4 is a diagrammatic plan view of an apparatus for processing lamp bases, generally illustrating the operations at various stations;

Fig. 5 is a fragmentary, sectional view taken at station "3" in Fig. 4 showing the application of the heat-protective coating;

Fig. 6 is a fragmentary, sectional view taken at station "4" in Fig. 4 showing the glassing operation;

25 Fig. 7 is a fragmentary, sectional view taken at station "6" in Fig. 4 showing the plunger-die operation for forming the poured glass into the desired configuration.

Although the principles of the invention are generally applicable to any type of lamp which desirably incorporates an aluminum base, the invention has particular reference with regard to bases for incandescent-type lamps and hence it has been so illustrated and will be so described.

With specific reference to the form of the invention

35 illustrated in the drawing, in Fig. 1 is shown an incandescent lamp 10 which generally comprises an envelope 12, base 14, lead conductors 16 hermetically sealed through a stem press 18 and supporting an incandescent filament 20 between their inwardly-extending extremities. One of the lead conductors is electrically connected to the aluminum base shell 22, which forms one contact electrode for the lamp. The other lead conductor is electrically connected to the centrally-disposed and electrically-conducting eyelet 24, which eyelet is

45 electrically insulated from aluminum base shell by an insulating button 26 which may be fabricated of glass. Such a lamp construction is generally well known.

In Fig. 2 is shown an aluminum base shell 22, before the glassing operation and such a base shell normally

50 has a generally-hollow-cylindrical and threaded configuration. The lower portion of the base shell forms an inwardly-projecting lip 28 which serves to hold the glass insulating button 26.

In Fig. 3 is shown the electrically-conducting eyelet

55 24 which may be punched from brass, for example, and which eyelet has a centrally-disposed aperture 30 forming a retaining lip which cooperates with the poured-glass insulating button 26 to retain the eyelet in position.

60 In Fig. 4 is shown a diagrammatic plan view of a base fabricating machine 32, modified slightly to provide for the application of the heat-protective coating as described herein. Such machines are normally designed to be indexed through a plurality of positions or work station

65 and at the station designated "1," the eyelet 24 is fed into the receiving mold by conventional techniques. At the station designated "2," the base shell 22 is fed into the receiving mold by conventional practices. At the station designated "3" the heat-protective coating is applied to at least the lower interior portions of the base

70 shell 22 and this coating may be applied as a spray by

a conventional atomizer. The heat-protective coating will be considered in detail hereinafter, but for a conventional medium-screw-type base, 0.2 cc. of heat-protective coating has been found to be adequate.

At the station designated "4," the molten glass is inserted or poured into the coated base shell 22 so as to cover the eyelet 24 and the lower interior surfaces of the base shell 22. This molten glass serves to separate the eyelet 24 from the base shell 22. Thereafter, excessive glass is blown from the upper surfaces of the molds and from between the molds at the glass-cutter stations designated "5" and this also serves to partially cool the poured glass. At the station designated "6," a glass plunger forms the interior surfaces of the poured glass into a generally conical configuration so that when the center lamp lead wire is later inserted into the base, it will be directed toward the aperture 30 in the centrally-disposed eyelet 24. At the station designated "7," an auxiliary glass plunger serves further to cool the poured glass in order to secure the eyelet 24 in the cooled glass button 26 and to secure the cooled glass button 26 in the base shell 22. At the station designated "8," a pin plunger removes any residue of glass from the aperture 30 of the centrally-disposed eyelet 24 and thereafter at the station designated "9," the completed bases are removed from the base-making machine 32. Such base-making machines as described herein are generally standard, with the exception of the heat-protective coating station designated "3."

In Fig. 5 is shown a base shell 22 and eyelet 24 contained in the mold 34 in position at the station designated "3" in Fig. 4 and the heat-protective coating is applied to at least the lower interior surfaces of the base shell 22 by means of a conventional atomizer 36. If desired, the heat-protective coating could be applied to the base shell 22 before the base shell was placed on the coating machine, but it is far more convenient automatically to apply this coating after the shell 22 has been placed into the mold 34.

The heat-protective coating principally comprises from 3 to 30% by weight sodium borophosphate, from 10% to 15% by weight sodium polyacrylate and from 55% to 87% by weight water. The molten glass which is poured into the base shell during the glassing operation may have a temperature of from 1185° C. to 1200° C., for example and, as noted hereinbefore, the aluminum under these conditions has a marked tendency to melt, at least in discrete portions. The heat-protective coating, as hereinbefore specified, forms a barrier or heat-protective layer between the molten glass and the aluminum base shell, substantially inhibiting any tendency for the aluminum base shell to melt.

Regarding the constituents of the heat-protective coating, sodium borophosphate has a high water of hydration and also has the property of encasing steam at high temperatures. The encased steam serves the dual function of providing an excellent insulating layer and also impairing the adherence of the sodium borophosphate for the base shell, which is highly desirable as will be explained hereinafter. A solution of sodium borophosphate in water, however, has a relatively low viscosity and will not adhere to the aluminum base shell in sufficient amounts to provide the proper degree of protection during the glassing operation.

Sodium polyacrylate has a high viscosity, is readily soluble in water, as is sodium borophosphate, and sodium polyacrylate has a high heat of vaporization. This material, however, tends to leave a carbonaceous residue after being heated, which residue is not readily removed by a water wash. This residue impairs the appearance of the completed base and also tends to form low-electrical-resistance paths.

When a mixture of sodium borophosphate and sodium polyacrylate in water solution is utilized as a heat-protective coating, the benefits of both of these constituents

are realized. Thus the admixture has sufficient viscosity (for example 32 c.p.s.) to provide an adequate amount of the heat-protective coating on the base and the steam which is encased by the sodium borophosphate renders

5 the admixture very poorly adherent to the aluminum base shell at high temperatures. Thus any coating residue is readily removed by a water wash. In addition, the individual constituents of the admixture both have a very high heat of vaporization, which improves the performance of the heat-protective coating.

If less than the indicated proportions comprising the admixture are used, the beneficial effects of the heat-protective coating are minimized. If the proportions of the sodium borophosphate and the polyacrylate are 15 greater than the maximum permissible amounts indicated hereinbefore, the viscosity of the resulting coating tends to be excessive and an excessive amount of the coating material is deposited. In addition, there is some tendency for residues where a relatively large amount of coating material has to be removed by a water wash and the adherence of the coating material for the aluminum base shell is somewhat increased, which also inhibits the removal of the coating material by a water wash. The preferred formulation for the heat-protective coating is 20 about 5% by weight sodium borophosphate, about 10% by weight sodium polyacrylate and about 85% by weight water.

It is also possible to incorporate small amounts of other additives into the heat-protective coating and if 30 desired, 5% by weight of ammonium polyacrylate may be substituted in place of an equivalent amount of water vehicle in the foregoing preferred specific embodiment. This somewhat increases the capacity for heat absorption of the coating, but such other small additives are 35 not necessary for good results. Other materials may be substituted in place of the ammonium polyacrylate additive, such as an equivalent weight of potassium silicate, for example.

In Fig. 6 is shown the glassing operation at the station designated "4" in Fig. 4. In this operation, a predetermined amount of molten glass is poured or inserted 40 into the coated base, such glass-pouring techniques being well known. As a specific example, in the case of a medium-screw type base, about 3.6 grams of glass may 45 be used. The glass may vary, but as a specific example, it may have the composition of 95% by weight cullet glass, 2.52% by weight  $MnO_2$ , 1.26% by weight  $KNO_3$ , 0.87% by weight  $(NH_4)_2SO_4$  and 0.35% by weight  $Cr_2O_3$ . The cullet glass, as used herein, has the composition 50 76.8% by weight  $SiO_2$ , 17.4% by weight  $Na_2O$ , 0.6% by weight  $K_2O$ , 0.4% by weight  $CaO$  and 3.6% by weight  $MgO$ . It should be understood that this glass is only given by way of specific example and other glasses and glassing compositions may be substituted.

55 In Fig. 7 is shown the glass-forming operation at the station designated "6" in Fig. 4. In this operation the glass-forming plunger 38 provides the interior surface of the poured glass with an inverted, generally-conical configuration in order that the center lead wire may be inserted into the eyelet by automatic equipment. The plunger station follows the glass pouring station at a sufficient time interval that the glass has partially cooled so that it is in a plastic state rather than a molten state. Thereafter, at the station designated "7" in Fig. 4, a conventional auxiliary glass plunger which is internally cooled with water, for example, is inserted into the base 60 in order to substantially cool the poured glass. An additional plunger, not shown, punches any residual glass which may remain within the centrally-disposed aperture 70 30 within the eyelet 24 in order that the center lead wire may be inserted therethrough during the lamp fabrication, and such a procedure is customary in the base-making art. The completed base is then discharged at the station designated "9" and is washed to remove all 75

dirt and other impurities as well as the residual heat-protective coating which remains.

In the cleaning process, any commercial cleaner may be used and the bases are placed into the cleaning solutions and agitated. This removes substantially all traces of dirt and other impurities as well as residual heat-protective coating. By way of specific examples of suitable cleaning solutions, the bases may be agitated in a dilute solution of nitric and sulphuric acid at a concentration of 40° to 45° Baumé. Alternatively, the bases may be cleaned with a 5% solution of ammonical soap or with a 3% to 5% lauryl-sulphate-type detergent, such as is commercially available under various trademarks. Other commercially-available cleaning solutions may be substituted for the specific examples given hereinbefore.

It may be desirable in some cases to dispense with the eyelet and to secure the lead wire to the exterior surface of the glass insulating button 26 by means of an epoxy-resin cement, for example. In such an embodiment, the procedures used in fabricating the base would be identical with those as outlined hereinbefore, except that the eyelet would not be placed into the mold.

The foregoing steps need not be carried out on the automatic equipment as outlined hereinbefore, but may be carried out by hand, if desired, although from the production standpoint, it is economically desirable to fabricate the bases on an automatic basis.

A further advantage of the heat-protective coating disclosed herein is that the aluminum base shells may be made thinner, if desired, thus eliminating the cost of using added aluminum in the base shells. In explanation, in the practices of the prior art it has been necessary to provide the aluminum base shell with a certain minimum thickness, for example .0125 inch for a medium-screw-type base, in order that the aluminum base shell has sufficient thermal capacity to absorb sufficient heat from the molten glass to prevent excessive melting of the aluminum. Even with this thickness of the aluminum base shell, considerable melting of the aluminum has been encountered. Where the heat-protective coating is interposed between the molten glass and the aluminum base shell, the thermal capacity required for the aluminum base shell is decreased and a medium-screw-type base shell having a thickness of only .0105 inch is generally satisfactory and will display substantially no melted portions.

It will be recognized that the objects of the invention have been achieved by providing a heat-protective coating for processing aluminum base shells as well as a method for processing aluminum base shells wherein any melting of the aluminum due to the molten glass is substantially eliminated. In addition, the aluminum base shells may be made thinner, if desired.

While in accordance with the patent statutes, one best-known embodiment of the invention has been illustrated and described in detail, it is to be particularly understood that the invention is not limited thereto or thereby.

I claim:

1. A heat-protective coating for processing aluminum base shells for lamps, said coating principally comprising from 3% to 30% by weight sodium borophosphate, from 10% to 15% by weight sodium polyacrylate, and from 55% to 87% by weight water.

2. A heat-protective coating for processing aluminum base shells for lamps, said coating principally comprising about 5% by weight sodium borophosphate, about 10% by weight sodium polyacrylate, and about 85% by weight water.

3. The method of glassing an aluminum base shell for a lamp, comprising applying to at least the lower interior surfaces of the aluminum base shell a heat-protective coating principally comprising from 3% to 30% by weight sodium borophosphate, from 10% to 15% by

weight sodium polyacrylate and from 55% to 87% by weight water, inserting a predetermined amount of molten glass into a mold containing said coated base shell to fill a selected portion of said coated base shell, cooling said base and said glass to secure said glass in said base, and thereafter cleaning said base with a cleaning solution to remove residual heat-protective coating.

4. The method of glassing an aluminum base shell for a lamp, comprising applying to at least the lower interior surfaces of the aluminum base shell a heat-protective coating principally comprising about 5% by weight sodium borophosphate, about 10% by weight sodium polyacrylate and about 85% by weight water, inserting a predetermined amount of molten glass into a mold containing said coated base shell to fill a selected portion of said coated base shell, cooling said base and said glass to secure said glass in said base, and thereafter cleaning said base with a water-vehicle cleaning solution to remove residual heat-protective coating.

5. The method of forming in an aluminum base shell for a lamp a glass insulating section having embedded therein a centrally-disposed and electrically-conducting eyelet insulated from said base shell, comprising placing said eyelet and said base shell into a mold and applying to at least the lower interior surfaces of said base shell a heat-protective coating principally comprising from 3% to 30% by weight sodium borophosphate, from 10% to 15% by weight sodium polyacrylate and from 55% to 87% by weight water, inserting into said mold a predetermined amount of molten glass covering said eyelet and the lower interior surfaces of said base shell and separating said eyelet from said base shell, partially cooling said glass, forming the upper surfaces of said partially cooled glass into a predetermined configuration, further cooling said formed glass to secure said eyelet in said cooled glass and to secure said cooled glass in said base shell, and thereafter cleaning said base with water-vehicle cleaning solution to remove residual heat-protective coating.

6. The method of forming in an aluminum base shell for a lamp a glass insulating section having embedded therein a centrally-disposed and electrically-conducting eyelet insulated from said base shell, comprising placing said eyelet and said base shell into a mold and applying to at least the lower interior surfaces of said base shell a heat-protective coating principally comprising about 5% by weight sodium borophosphate, about 10% by weight sodium polyacrylate and about 85% by weight water, inserting into said mold a predetermined amount of molten glass covering said eyelet and the lower interior surfaces of said base shell and separating said eyelet from said base shell, partially cooling said glass, forming the upper surfaces of said partially cooled glass into a predetermined configuration, further cooling said formed glass to secure said eyelet in said cooled glass and to secure said cooled glass in said base shell, and thereafter cleaning said base with a water-vehicle cleaning solution to remove residual heat-protective coating.

#### 60 References Cited in the file of this patent

#### UNITED STATES PATENTS

|           |                     |               |
|-----------|---------------------|---------------|
| 1,011,586 | Criggal             | Dec. 12, 1911 |
| 1,976,679 | Fikenstscher et al. | Oct. 9, 1934  |
| 2,158,044 | Haller              | May 9, 1939   |
| 2,387,865 | Kleeck              | Oct. 30, 1945 |
| 2,413,146 | Larson              | Dec. 24, 1946 |
| 2,439,395 | Leatherman          | Apr. 13, 1948 |
| 2,480,790 | Truhlar             | Aug. 30, 1949 |
| 2,538,589 | Poje                | Jan. 16, 1951 |

#### FOREIGN PATENTS

|         |        |              |
|---------|--------|--------------|
| 797,345 | France | Feb. 8, 1936 |
|---------|--------|--------------|